



US005718779A

**United States Patent** [19]

Fukai et al.

[11] Patent Number: **5,718,779**[45] Date of Patent: **Feb. 17, 1998**

[54] **METHOD FOR MANUFACTURING A +  $\beta$  TYPE TITANIUM ALLOY PLATE HAVING SMALL ANISOTROPY**

[75] Inventors: **Hideaki Fukai; Toru Izawa; Takayuki Kobayashi**, all of Tokyo, Japan

[73] Assignee: **NKK Corporation, Japan**

[21] Appl. No.: **747,636**

[22] Filed: **Nov. 13, 1996**

[30] **Foreign Application Priority Data**

Nov. 14, 1995 [JP] Japan ..... 7-295544

[51] Int. Cl. <sup>6</sup> ..... **C22C 1/18**

[52] U.S. Cl. ..... **148/670; 148/671**

[58] Field of Search ..... **148/668, 669, 148/670, 671**

[56] **References Cited**

**U.S. PATENT DOCUMENTS**

4,581,077 4/1986 Sakuyama et al. ..... 148/670  
4,830,683 5/1989 Farguson ..... 148/670  
4,871,400 10/1989 Shindo et al. ..... 148/671

**FOREIGN PATENT DOCUMENTS**

63-130753 6/1988 Japan .....  
2158373 11/1985 United Kingdom .

**OTHER PUBLICATIONS**

M.J. Donachie Jr.: "Titanium A Technical Guide" 1988, American Society for Metals, Metals Park, Ohio, pp. 47-50.

*Primary Examiner*—John Sheehan  
*Attorney, Agent, or Firm*—Akin, Gump, Strauss, Hauer & Feld, L.L.P.

[57] **ABSTRACT**

A method for manufacturing an  $\alpha+\beta$  type titanium alloy plate having a small anisotropy in strength by subjecting an  $\alpha+\beta$  type titanium alloy slab to a hot-rolling, which comprises: the hot-rolling comprising a cross-rolling which comprises a hot-rolling in a L-direction and a hot-rolling in a C-direction, the L-direction being a final rolling direction in the hot-rolling and the C-direction being a direction at right angles to the L-direction; and controlling the cross-rolling so that a value of an overall cross ratio of rolling ( $CR_{total}$ ) determined by means of the following formula is kept within a range of from 0.5 to 2.0:

$$CR_{total} = (CR_1)^{0.6} \times (CR_2)^{0.4} \times (CR_3)^{1.0}$$

where,  $CR_1$  is a cross ratio of rolling within a rolling temperature region of from under  $T\beta$  °C. to  $T\beta$  °C.-50° C.,  $CR_2$  is a cross ratio of rolling within a rolling temperature region of from under  $T\beta$  °C.-50° C. to  $T\beta$  °C.-150° C.,  $CR_3$  is a cross ratio of rolling within a rolling temperature region of under  $T\beta$  °C.-150° C., and  $T\beta$  °C. is a  $\beta$ -transformation temperature of an  $\alpha+\beta$  type titanium alloy.

**7 Claims, 1 Drawing Sheet**



FIG. 1



**METHOD FOR MANUFACTURING A +  $\beta$  TYPE TITANIUM ALLOY PLATE HAVING SMALL ANISOTROPY**

**REFERENCE TO PATENTS, APPLICATIONS AND PUBLICATIONS PERTINENT TO THE INVENTION**

As far as we know, there is available the following prior art document pertinent to the present invention:

Japanese Patent Provisional Publication No. JP-A-63-130,753 published on Jun. 2, 1988.

The contents of the prior art disclosed in the above-mentioned prior art document will be discussed under the heading of "BACKGROUND OF THE INVENTION".

**BACKGROUND OF THE INVENTION**

**1. Field of the Invention**

The present invention relates to a method for manufacturing an  $\alpha+\beta$  type titanium alloy plate, and more particularly, to a method for manufacturing an  $\alpha+\beta$  type titanium alloy plate having a small anisotropy in strength.

**2. Related Art Statement**

It is the conventional practice to manufacture an  $\alpha+\beta$  type titanium alloy plate having a prescribed thickness by slab-forging or slab-rolling an  $\alpha+\beta$  type titanium alloy material such as an  $\alpha+\beta$  type titanium alloy ingot into an  $\alpha+\beta$  type titanium alloy slab, and then hot-rolling the thus prepared  $\alpha+\beta$  type titanium alloy slab.

For hot-rolling an  $\alpha+\beta$  type titanium alloy slab, there is a temperature region suitable for the hot-rolling from the point of view of hot-workability. Therefore, when hot-rolling an  $\alpha+\beta$  type titanium alloy slab having a large cross-section into an  $\alpha+\beta$  type titanium alloy plate, or when hot-rolling an  $\alpha+\beta$  type titanium alloy slab into a thin  $\alpha+\beta$  type titanium alloy plate (hereinafter referred to as the "thin-plate rolling"), it is difficult to manufacture a product having a desired thickness by a method for manufacturing an  $\alpha+\beta$  type titanium alloy plate, which comprises once heating an  $\alpha+\beta$  type titanium alloy slab, and then hot-rolling several times the thus once heated slab (hereinafter referred to as the "single-heat rolling"). In such a case, therefore, it is necessary to adopt a method for manufacturing an  $\alpha+\beta$  type titanium alloy plate, which comprises reheating the single-heat rolled  $\alpha+\beta$  type titanium alloy slab, and then hot-rolling several times the thus reheated slab (hereinafter referred to as the "multi-heat rolling").

When conducting the foregoing thin-plate rolling, furthermore, it is the common practice to apply a manner of rolling known as the pack-rolling which comprises covering at least an upper surface and a lower surface of an  $\alpha+\beta$  type titanium alloy slab with a carbon steel sheet, and hot-rolling the  $\alpha+\beta$  type titanium alloy slab thus covered with the carbon steel sheet.

When manufacturing a titanium plate, in general, a crystal texture is formed in a titanic slab during the hot-rolling thereof not only in the case of the  $\alpha+\beta$  type titanium alloy, but also in the case of an  $\alpha$  type titanium alloy or pure titanium. Consequently, anisotropy in strength is produced in the resultant product. For the purpose of restraining the production of anisotropy in strength, there is known a method comprising using a cross-rolling as the hot-rolling and controlling a cross ratio of rolling.

For example, Japanese Patent Provisional publication No. JP-A-63-130,753 published on Jun. 2, 1988 discloses a method for manufacturing a pure titanium plate having a small anisotropy, which comprises:

heating a pure titanium material having a thickness  $t_0$  to a  $\beta$ -phase temperature region not exceeding 970° C., then slab-rolling the thus heated pure titanium material at a draft of at least 30% into a pure titanium slab having a thickness  $t_1$ , then cooling the resultant slab, then reheating the resultant cold slab to a temperature not exceeding a  $\beta$ -transformation temperature, then subjecting the thus reheated pure titanium slab to a hot-rolling comprising a cross-rolling in a rolling direction, in which a final rolling direction in the hot-rolling is at right angles to a rolling direction in the slab-rolling, while keeping a cross ratio of rolling  $[(t_1/t_2)/(t_0/t_1)]$  within a range of from 0.5 to 3.0, to prepare a pure titanium plate having a thickness  $t_2$ , then cooling the resultant pure titanium plate, and then annealing the thus cooled pure titanium plate (hereinafter referred to as the "prior art 1").

In addition, there is available a common method for manufacturing an  $\alpha+\beta$  type titanium alloy plate, which comprises cross-rolling an  $\alpha+\beta$  type titanium alloy slab to minimize anisotropy in strength (hereinafter referred to as the "prior art 2").

The prior arts 1 and 2 described above, however, involve the following problems:

When hot-rolling an  $\alpha+\beta$  type titanium alloy slab, and if a temperature region of the hot-rolling differs, an  $\alpha$ -phase and a  $\beta$ -phase in the hot-rolled  $\alpha+\beta$  type titanium alloy slab have different volume fractions. Even when the  $\alpha+\beta$  type titanium alloys have the same chemical composition, therefore, the extent of the effect of a draft on anisotropy in strength varies depending upon temperature regions of the hot-rolling of the  $\alpha+\beta$  type titanium alloy slabs. When hot-rolling an  $\alpha+\beta$  type titanium alloy slab, therefore, it is impossible to satisfactorily restrain anisotropy in strength of an  $\alpha+\beta$  type titanium alloy plate by means of a cross ratio of rolling determined simply only from a thickness of the  $\alpha+\beta$  type titanium alloy slab before the hot-rolling and a thickness of the  $\alpha+\beta$  type titanium alloy plate after the completion of the hot-rolling, as in the prior arts 1 and 2.

Under these circumstances, there is a strong demand for development of a method for manufacturing an  $\alpha+\beta$  type titanium alloy plate having a small anisotropy in strength, but such a method has not as yet been proposed.

**SUMMARY OF THE INVENTION**

An object of the present invention is therefore to provide a method for manufacturing an  $\alpha+\beta$  type titanium alloy plate excellent in isotropy with a small anisotropy in strength.

In accordance with one of the features of the present invention, there is provided a method for manufacturing an  $\alpha+\beta$  type titanium alloy plate having a small anisotropy in strength by subjecting an  $\alpha+\beta$  type titanium alloy slab to a hot-rolling, which comprises:

said hot-rolling comprising a cross-rolling which comprises a hot-rolling in an L-direction and a hot-rolling in a C-direction, said L-direction being a final rolling direction in said hot-rolling and said C-direction being a direction at right angles to said L-direction; and

controlling said cross-rolling so that a value of an overall cross ratio of rolling ( $CR_{total}$ ) determined by means of the following formula is kept within a range of from 0.5 to 2.0:

$$CR_{total} = (CR_1)^{0.6} \times (CR_2)^{0.8} \times (CR_3)^{1.0}$$

where,

$CR_{total}$ : overall cross ratio of rolling,

CR<sub>1</sub>: cross ratio of rolling within a rolling temperature region of from under T<sub>β</sub> °C. to T<sub>β</sub> °C.-50° C.,

CR<sub>2</sub>: cross ratio of rolling within a rolling temperature region of from under T<sub>β</sub> °C.-50° C. to T<sub>β</sub> °C.-150° C.,

CR<sub>3</sub>: cross ratio of rolling within a rolling temperature region of under T<sub>β</sub> °C.-150° C., and

T<sub>β</sub> °C.: β-transformation temperature of an α+β type titanium alloy.

#### BRIEF DESCRIPTION OF THE DRAWING

FIG. 1 is a graph illustrating the effect of an overall cross ratio of rolling (CR<sub>total</sub>) determined by means of the following formula:

$$CR_{total} = (CR_1)^{0.6} \times (CR_2)^{0.8} \times (CR_3)^{1.0}$$

on anisotropy in strength of an α+β type titanium alloy plate.

#### DETAILED DESCRIPTION OF PREFERRED EMBODIMENTS

From the above-mentioned point of view, extensive studies were carried out to develop a method for manufacturing an α+β type titanium alloy plate excellent in isotropy with a small anisotropy in strength.

As a result, the following findings were obtained: Production of anisotropy in strength of an α+β type titanium alloy plate is attributable to the fact that, during the hot-rolling of an α+β type titanium alloy slab, an α-phase crystal texture is formed therein. In the hot-rolled α+β type titanium alloy slab, however, an α-phase and a β-phase have different volume fractions, depending upon a temperature region of the hot-rolling. Therefore, the extent of the effect of a cross ratio of rolling on anisotropy in strength depends upon a temperature region of the hot-rolling of the α+β type titanium alloy slab. Furthermore, anisotropy in strength of the α+β type titanium alloy slab produced during the preceding hot-rolling, still remains after reheating thereof. Therefore, a trial, as in the prior arts 1 and 2, to restrain anisotropy in strength of an α+β type titanium alloy plate by means of a cross ratio of rolling determined simply only from a thickness of the α+β type titanium alloy slab before the hot-rolling and a thickness of the α+β type titanium alloy plate after the completion of the hot-rolling, without taking account of a volume fraction of an α-phase in the α+β type titanium alloy slab, which varies depending upon a temperature region of the hot-rolling, does not give a satisfactory result.

Then, further studies were carried out, paying attention to the fact that the extent of the effect of a cross ratio of rolling on anisotropy in strength varies depending upon temperature regions of the hot-rolling of the α+β type titanium alloy slab. As a result, the following findings were obtained: It is possible to manufacture an α+β type titanium alloy plate having a small anisotropy in strength by dividing a temperature region of the hot-rolling into a plurality of appropriate rolling temperature regions, determining an overall cross ratio of rolling (CR<sub>total</sub>) on the basis of a cross ratio of rolling determined for each of the thus divided individual rolling temperature regions, and cross-rolling an α+β type titanium alloy slab so as to keep a value of the overall cross ratio of rolling (CR<sub>total</sub>) thus determined within a prescribed range.

The present invention was developed on the basis of the foregoing findings, and a method of the present invention for manufacturing an α+β type titanium alloy plate having a

small anisotropy in strength by subjecting an α+β type titanium alloy slab to a hot-rolling, which comprises:

said hot-rolling comprising a cross-rolling which comprises a hot-rolling in an L-direction and a hot-rolling in a C-direction, said L-direction being a final rolling direction in said hot-rolling and said C-direction being a direction at right angles to said L-direction; and

controlling said cross-rolling so that a value of an overall cross ratio of rolling (CR<sub>total</sub>) determined by means of the following formula is kept within a range of from 0.5 to 2.0:

$$CR_{total} = (CR_1)^{0.6} \times (CR_2)^{0.8} \times (CR_3)^{1.0}$$

where,

CR<sub>total</sub>: overall cross ratio of rolling.

CR<sub>1</sub>: cross ratio of rolling within a rolling temperature region of from under T<sub>β</sub> °C. to T<sub>β</sub> °C.-50° C.,

CR<sub>2</sub>: cross ratio of rolling within a rolling temperature region of from under T<sub>β</sub> °C.-50° C. to T<sub>β</sub> °C.-150° C.,

CR<sub>3</sub>: cross ratio of rolling within a rolling temperature region of under T<sub>β</sub> °C.-150° C., and

T<sub>β</sub> °C.: β-transformation temperature of an α+β type titanium alloy.

In the method of the present invention, the term of a cross ratio of rolling is defined as follows: When a final rolling direction in the hot-rolling of an α+β type titanium alloy slab is referred to as an L-direction, and a direction at right angles to the L-direction is referred to as a C-direction, and when the thickness of the titanium alloy slab is reduced from A<sub>0</sub> to A<sub>1</sub> in the hot-rolling in the C-direction, and then, the thickness of the titanium alloy slab is reduced from A<sub>1</sub> to A<sub>2</sub> in the hot-rolling in the L-direction, the cross ratio of rolling is expressed by the following formula:

---


$$\begin{aligned} \text{Cross ratio of rolling} \\ &= (\text{draft of rolling in the L-direction}) \\ &\quad (\text{draft of rolling in the C-direction}) \\ &= (A_1/A_2)/(A_0/A_1) \end{aligned} \quad (1)$$


---

The formula (1) can be rewritten as follows:

$$CR_{total} = (A_1/A_0) \times (A_1/A_2) \quad (2)$$

The formula (2) is used as the general formula of the cross ratio of rolling.

In the method of the present invention, an overall cross ratio of rolling (CR<sub>total</sub>) is determined by the following formula (3):

$$CR_{total} = (CR_1)^{0.6} \times (CR_2)^{0.8} \times (CR_3)^{1.0} \quad (3)$$

where,

CR<sub>total</sub>: overall cross ratio of rolling.

CR<sub>1</sub>: cross ratio of rolling within a rolling temperature region of from under T<sub>β</sub> °C. to T<sub>β</sub> °C.-50° C.,

CR<sub>2</sub>: cross ratio of rolling within a rolling temperature region of from under T<sub>β</sub> °C.-50° C. to T<sub>β</sub> °C.-150° C.,

CR<sub>3</sub>: cross ratio of rolling within a rolling temperature region of under T<sub>β</sub> °C.-150° C., and

T<sub>β</sub> °C.: β-transformation temperature of an α+β type titanium alloy,

and CR<sub>1</sub>, CR<sub>2</sub> and CR<sub>3</sub> are determined from the general formula (2) above.

Now, a first embodiment of the present invention is described below.

In the first embodiment of the present invention, a hot-rolling of an  $\alpha+\beta$  type titanium alloy slab comprises a rough-rolling and a finish-rolling. Table 1 shows a pass schedule of the hot-rolling in the first embodiment of the present invention, i.e., a thickness reduction, a rolling temperature region, a rolling direction, a timing of turning of the rolling direction by  $90^\circ$  and a cross ratio of rolling in individual steps of the rough-rolling and the finish-rolling.

#### Finish-rolling:

The thus prepared rough-rolled slab having a thickness  $t_4$  is reheated to a temperature of  $T\beta$  °C.-20°C., then the thus reheated rough-rolled slab is reduced from thickness  $t_4$  to  $t_5$  in the same rolling direction as the final rolling direction in the rough-rolling within a rolling temperature region of from under  $T\beta$  °C. to  $T\beta$  °C.-50°C., then the resultant slab is reduced from thickness  $t_5$  to  $t_6$  within a rolling temperature region of from under  $T\beta$  °C.-50°C. to  $T\beta$  °C.-150°C. Then the rolling direction of the slab is turned by  $90^\circ$  C. to resume

TABLE 1

| <u>Rough-rolling</u>       |                          |                                                 |
|----------------------------|--------------------------|-------------------------------------------------|
| Thickness                  |                          |                                                 |
| Rolling temperature region |                          |                                                 |
| Rolling direction          |                          |                                                 |
| Cross ratio of rolling     |                          |                                                 |
| $t_0$                      | $t_1$                    | $t_2$                                           |
| under $T\beta$ °C.         | under $T\beta$ °C.-50°C. | under $T\beta$ °C.-50°C. to $T\beta$ °C.-150°C. |
| L-direction                |                          |                                                 |
| $CR_1^{0.6}$               | $CR_2^{0.8}$             | $CR_3^{1.0}$                                    |
| $t_3$                      | $t_4$                    |                                                 |
| $90^\circ$ -turning        |                          |                                                 |
| <u>Finish-rolling</u>      |                          |                                                 |
| Thickness                  |                          |                                                 |
| Rolling temperature region |                          |                                                 |
| Rolling direction          |                          |                                                 |
| Cross ratio of rolling     |                          |                                                 |
| $t_1$                      | $t_5$                    | $t_6$                                           |
| under $T\beta$ °C.         | under $T\beta$ °C.-50°C. | under $T\beta$ °C.-50°C. to $T\beta$ °C.-150°C. |
| C-direction                |                          |                                                 |
| $CR_1^{0.6}$               | $CR_2^{0.8}$             | $CR_3^{1.0}$                                    |
| $t_7$                      | $t_8$                    | $t_9$                                           |
| $90^\circ$ -turning        |                          |                                                 |

In the first embodiment of the present invention, as shown in Table 1, when a final rolling direction in a finish-rolling is referred to as an L-direction, and a direction at right angles to the L-direction is referred to as a C-direction, the first rolling direction in the finish-rolling is the same as the final rolling direction in the rough-rolling, i.e., the C-direction.

In the first embodiment of the present invention, an  $\alpha+\beta$  type titanium alloy slab is soaked at a temperature of  $T\beta$  °C.-20°C. ( $T\beta$  °C. means a  $\beta$ -transformation temperature of an  $\alpha+\beta$  type titanium alloy), and the thus soaked slab is subjected to a rough-rolling, and then to a finish-rolling, as described below.

#### Rough Rolling:

The slab soaked at a temperature of  $T\beta$  °C.-20°C. is reduced from thickness  $t_0$  to  $t_1$  within a rolling temperature region of from under  $T\beta$  °C. to  $T\beta$  °C.-50°C., and then the resultant slab is reduced from thickness  $t_1$  to  $t_2$  within a rolling temperature region of from under  $T\beta$  °C.-50°C. to  $T\beta$  °C.-150°C. Then the rolling direction of the slab is turned by  $90^\circ$  to resume the rough-rolling, then the slab is reduced from thickness  $t_2$  to  $t_3$  within a rolling temperature region of from under  $T\beta$  °C.-50°C. to  $T\beta$  °C.-150°C., and then the resultant slab is reduced from thickness  $t_3$  to  $t_4$  within a rolling temperature region of from under  $T\beta$  °C.-50°C. to  $T\beta$  °C.-150°C., thereby preparing a rough-rolled slab having a thickness  $t_4$ .

40 the finish-rolling, then the slab is reduced from thickness  $t_6$  to  $t_7$  within a rolling temperature region of from under  $T\beta$  °C.-50°C. to  $T\beta$  °C.-150°C., and then the resultant slab is reduced from thickness  $t_7$  to  $t_8$  in the L-direction within a rolling temperature region of under  $T\beta$  °C.-150°C., thereby 45 manufacturing an  $\alpha+\beta$  type titanium alloy plate having a thickness  $t_8$ .

A cross ratio of rolling in the above-mentioned rough-rolling and finish-rolling is determined in accordance with the following formula:

50 Cross Ratio of Rolling in Rough-rolling:

$$(CR_1)^{0.6} = (t_0/t_1)^{0.6}$$

$$(CR_2)^{0.8} = (t_1/t_2)^{0.8} \times (t_3/t_2)^{0.8}, \text{ and}$$

$$(CR_3)^{1.0} = (t_4/t_3)^{1.0};$$

Cross Ratio in Finish-rolling:

$$(CR_1)^{0.6} = (t_6/t_7)^{0.6},$$

$$(CR_2)^{0.8} = (t_7/t_8)^{0.8} \times (t_8/t_6)^{0.8}, \text{ and}$$

$$(CR_3)^{1.0} = (t_8/t_7)^{1.0}.$$

65 Accordingly, an overall cross ratio of rolling ( $CR_{total}$ ) in the first embodiment of the present invention is determinable by means of the following formula (4):

$$\begin{aligned}
 CR_{total} &= (CR_1)^{0.6} \times (CR_2)^{0.8} \times (CR_3)^{1.0} \\
 &= [(CR_1)^{0.6} \times (CR_2)^{0.8} \times (CR_3)^{1.0} \text{ in rough-rolling}] \times \\
 &\quad [(CR_1)^{0.6} \times (CR_2)^{0.8} \times (CR_3)^{1.0} \text{ in finish-rolling}] \\
 &= [(t_1/t_1)^{0.6} \times \{(t_2/t_1)^{0.8} \times (t_3/t_2)^{0.8}\} \times \\
 &\quad (t_4/t_3)^{1.0}] \times [(t_2/t_1)^{0.6} \times \{(t_3/t_2)^{0.8} \times \\
 &\quad (t_4/t_3)^{0.8}\} \times (t_2/t_1)^{1.0}]
 \end{aligned} \tag{4}$$

where,

$CR_1$ : cross ratio of rolling within a rolling temperature region of from under  $T\beta$  °C. to  $T\beta$  °C.-50° C..

$CR_2$ : cross ratio of rolling within a rolling temperature region of from under  $T\beta$  °C.-50° C. to  $T\beta$  °C.-150° C..

$CR_3$ : cross ratio of rolling within a rolling temperature region of under  $T\beta$  °C.-150° C., and

$T\beta$  °C.:  $\beta$ -transformation temperature of an  $\alpha+\beta$  type titanium alloy.

In the first embodiment of the present invention, the hot-rolling comprising the rough-rolling and the finish-rolling of the  $\alpha+\beta$  type titanium alloy slab, is controlled so as to keep a value of the overall cross ratio of rolling ( $CR_{total}$ ) determined by means of the foregoing formula (4) within a range of from 0.5 to 2.0.

Now, a second embodiment of the present invention is described.

In the first embodiment of the present invention, as described above, the first rolling direction in the finish-rolling is the same as the final rolling direction in the rough-rolling. In the second embodiment of the present invention, in contrast, the first rolling direction in the finish-rolling is at right angles to the final rolling direction in the rough-rolling. The second embodiment of the present invention differs from the first embodiment of the present invention only in the foregoing point.

An overall cross ratio of rolling ( $CR_{total}$ ) in the second embodiment of the present invention is determined by means of the following formula (5):

$$\begin{aligned}
 CR_{total} &= \\
 &[(t_1/t_1)^{0.6} \times \{(t_2/t_1)^{0.8} \times (t_2/t_3)^{0.8}\} \times \\
 &\quad (t_3/t_4)^{1.0}] \times [(t_2/t_1)^{0.6} \times \{(t_3/t_2)^{0.8} \times \\
 &\quad (t_4/t_3)^{0.8}\} \times (t_2/t_1)^{1.0}]
 \end{aligned} \tag{5}$$

In the second embodiment of the present invention, the hot-rolling comprising the rough-rolling and the finish-rolling of the  $\alpha+\beta$  type titanium alloy slab, is controlled so as to keep a value of the overall cross ratio of rolling ( $CR_{total}$ ) determined by means of the foregoing formula (5) within a range of from 0.5 to 2.0.

In the method of the present invention, the temperature region of the hot-rolling of the  $\alpha+\beta$  type titanium alloy slab is divided into the following three rolling temperature regions:

Rolling temperature region A: a rolling temperature region of from under  $T\beta$  °C. to  $T\beta$  °C.-50° C.,

Rolling temperature region B: a rolling temperature region of from under  $T\beta$  °C.-50° C. to  $T\beta$  °C.-150° C., and

Rolling temperature region C: a rolling temperature region of under  $T\beta$  °C.-150° C.

and the cross ratio of rolling ( $CR_1$ ,  $CR_2$  and  $CR_3$ ) is determined for each of these rolling temperature regions A, B and C, and the overall cross ratio of rolling ( $CR_{total}$ ) is determined on the basis of  $CR_1$ ,  $CR_2$  and  $CR_3$ . The reasons therefor are as follows.

As previously described above, production of anisotropy in strength of an  $\alpha+\beta$  type titanium alloy plate is attributable

to the fact that, during the hot-rolling of an  $\alpha+\beta$  type titanium alloy slab, an  $\alpha$ -phase crystal texture is formed therein, and in the  $\alpha+\beta$  type titanium alloy slab, an  $\alpha$ -phase and a  $\beta$ -phase have different volume fractions, depending upon a temperature region of the hot-rolling.

More specifically, in a high-temperature region near the  $\beta$ -transformation temperature ( $T\beta$  °C.), the  $\alpha$ -phase having an important effect on the formation of a crystal texture has only a small volume fraction. In contrast, the  $\alpha$ -phase has a large volume fraction in a low-temperature region. In the hot-rolling at a low temperature, furthermore, the  $\alpha$ -phase is more seriously deformed and more crystal textures of the  $\alpha$ -phase are formed. As a result, in the hot-rolling in a relatively low-temperature region, more crystal textures of the  $\alpha$ -phase which has an important effect on production of anisotropy are formed. When restraining production of anisotropy in strength by means of the cross-rolling, therefore, the effect of the cross ratio of rolling is smaller in the high-temperature region near  $T\beta$  °C., and larger in the low-temperature region. For this reason, it is necessary to place a weight on the cross ratio of rolling in response to the rolling temperature region.

In the method of the present invention, such weights as  $(CR_1)^{0.6}$ ,  $(CR_2)^{0.8}$  and  $(CR_3)^{1.0}$  are placed on the cross ratios of rolling for the three rolling temperature regions A, B and C for the above-mentioned reason.

Therefore, the overall cross ratio of rolling ( $CR_{total}$ ) determined by means of the following formula (3):

$$CR_{total} = (CR_1)^{0.6} \times (CR_2)^{0.8} \times (CR_3)^{1.0} \tag{3}$$

is most appropriately correlated with anisotropy in strength of the  $\alpha+\beta$  type titanium plate.

Now, the reason of limiting a value of the above-mentioned overall cross ratio of rolling ( $CR_{total}$ ) within a range of from 0.5 to 2.0 in the method of the present invention, is described below.

FIG. 1 is a graph illustrating the effect of an overall cross ratio of rolling ( $CR_{total}$ ) determined by means of the following formula (3):

$$CR_{total} = (CR_1)^{0.6} \times (CR_2)^{0.8} \times (CR_3)^{1.0} \tag{3}$$

on anisotropy in strength of an  $\alpha+\beta$  type titanium alloy plate.

The ordinate in FIG. 1 represents anisotropy in strength of the  $\alpha+\beta$  type titanium alloy plate. This anisotropy in strength is expressed, when a final rolling direction of the hot-rolling of an  $\alpha+\beta$  type titanium alloy slab is referred to as a L-direction, and a direction at right angles to the L-direction is referred to as a C-direction, by a ratio  $[PS(L)/PS(C)]$  of a 0.2% proof stress in the L-direction (hereinafter referred to as "PS(L)") to a 0.2% proof stress in the C-direction (hereinafter referred to as "PS(C)"), obtained by means of a tensile test.

In FIG. 1, the mark ● represents an  $\alpha+\beta$  type titanium alloy slab comprising a Ti-4.5Al-3V-2Mo-2Fe alloy, and the mark ○ represents an  $\alpha+\beta$  type titanium alloy slab comprising a Ti-6Al-4V alloy.

As is clear from FIG. 1, there is a close correlation between the overall cross ratio ( $CR_{total}$ ) and anisotropy in strength  $[PS(L)/PS(C)]$ .

When an absolute value of a difference between the 0.2% proof stress in the L-direction  $[PS(L)]$  and the 0.2% proof stress in the C-direction  $[PS(C)]$  of the  $\alpha+\beta$  type titanium alloy plate is over 20% of the 0.2% proof stress in the L-direction  $[PS(L)]$  or the 20% proof stress in the

C-direction [PS(C)], undesirable non-uniform deformations tend to be easily caused by anisotropy in strength upon working the  $\alpha+\beta$  type titanium alloy plate. In order to minimize anisotropy in strength, therefore, it is necessary to limit a value of [PS(L)/PS(C)] within a range of from 0.80 to 1.20.

On the other hand, the overall cross ratio of rolling ( $CR_{total}$ ) can be adjusted in a pass schedule of the hot-rolling. Anisotropy in strength can be restrained by adjusting the overall cross ratio of rolling ( $CR_{total}$ ). As is clear from FIG. 1, therefore, in order to minimize anisotropy in strength of an  $\alpha+\beta$  type titanium alloy plate, a value of the overall cross ratio of rolling ( $CR_{total}$ ) should be limited within a range of from 0.5 to 2.0.

Now, the method of the present invention is described further in detail by means of examples while comparing with examples for comparison.

## EXAMPLES

### Example 1

An alloy comprising a Ti-4.5Al-3V-2Mo-2Fe alloy was employed as an  $\alpha+\beta$  type titanium alloy. Since this titanium alloy has a  $\beta$ -transformation temperature ( $T\beta$  °C.) of 900° C., the temperature region of the hot-rolling of the titanium alloy slab was divided, in Example 1, into three rolling temperature regions of (1) from under 900° C. to 850° C., (2) from under 850° C. to 750° C., and (3) under 750° C.

First, an  $\alpha+\beta$  type titanium alloy slab having a thickness of 200 mm and the above-mentioned chemical composition was soaked at a temperature of 880° C., and then rough-rolled in accordance with a pass schedule shown in Table 2. More particularly, the titanium alloy slab thus soaked was reduced from a thickness of 200 mm to 122 mm within a rolling temperature region of from under 880° C. to 850° C., and then was reduced from a thickness of 122 mm to 62 mm within a rolling temperature region of from under 850° C. to 750° C. Then the rolling direction of the slab was turned by 90° to resume the rough-rolling, then the slab was reduced from a thickness of 62 mm to 44 mm within a rolling temperature region of from under 850° C. to 750° C., and then the resultant slab was reduced from a thickness of from 44 mm to 20 mm within a rolling temperature region of under 750° C., thereby preparing a rough-rolled slab having a thickness of 20 mm.

The thus prepared rough-rolled slab having a thickness of 20 mm was reheated to a temperature of 880° C., and then finish-rolled in accordance with a pass schedule shown in Table 2. More specifically, the rough-rolled slab having a thickness of 20 mm was reduced from a thickness of 20 mm to 17 mm in the same rolling direction as the final rolling direction in the foregoing rough-rolling within a rolling temperature region of from under 880° C. to 850° C., and then was reduced from a thickness of 17 mm to 9 mm within a rolling temperature region of from under 850° C. to 750° C. Then the rolling direction of the slab was turned by 90° to resume the finish-rolling, then the slab was reduced from a thickness of 9 mm to 7 mm within a rolling temperature

region of from under 850° C. to 750° C., and then the resultant slab was reduced from a thickness of 7 mm to 4 mm in the L-direction within a rolling temperature region of under 750° C., thereby obtaining an  $\alpha+\beta$  type titanium alloy plate having a thickness of 4 mm. Subsequently, the resultant titanium alloy plate was cooled, and then annealed at a temperature of 720° C. for a period of time of an hour, thereby preparing an  $\alpha+\beta$  type titanium alloy plate having a thickness of 4 mm within the scope of the present invention (hereinafter referred to as the "sample of the invention") No. 1.

In the above-mentioned rough-rolling and finish-rolling, a value of the overall cross ratio of rolling ( $CR_{total}$ ) was kept within a range of from 0.5 to 2.0, which was within the scope of the present invention.

Then, while keeping a value of the overall cross ratio of rolling ( $CR_{total}$ ) within a range of from 0.5 to 2.0, which was within the scope of the present invention,  $\alpha+\beta$  type titanium alloy slabs having the same chemical composition and the same thickness as those in the sample of the invention No.

20 1, were rough-rolled and then finish-rolled in accordance with pass schedules shown in Tables 2 to 4, and 6 in the same manner as described above, thereby obtaining  $\alpha+\beta$  type titanium alloy plates having a thickness of 4 mm. Then the resultant titanium alloy plates were cooled, and then annealed at a temperature of 720° C. for a period of time of an hour, thereby preparing  $\alpha+\beta$  type titanium alloy plates having a thickness of 4 mm within the scope of the present invention (hereinafter referred to as the "samples of the invention") Nos. 2 to 6, 9 and 10.

30 Then, while keeping a value of the overall cross ratio of rolling ( $CR_{total}$ ) within a range of from 0.5 to 2.0, which was within the scope of the present invention,  $\alpha+\beta$  type titanium alloy slabs having the same chemical composition and the same thickness as those of the sample of the invention No. 1, were subjected to the single-heat rolling in accordance with pass schedules shown in Table 7, thereby obtaining  $\alpha+\beta$  type titanium alloy plates having a thickness of 20 mm. Then the resultant titanium alloy plates were cooled, and then annealed at a temperature of 720° C. for a period of time of an hour, thereby preparing  $\alpha+\beta$  type titanium alloy plates having a thickness of 20 mm within the scope of the present invention (hereinafter referred to as the "samples of the invention") Nos. 11 and 12.

45 Subsequently, for comparison purposes,  $\alpha+\beta$  type titanium alloy slabs having the same chemical composition and the same thickness as those of the sample of the invention No. 1, were rough-rolled and then finish-rolled in accordance with pass schedules shown in Tables 5 and 7 in the same manner as described in the sample of the invention No. 1, while keeping a value of the overall cross ratio of rolling ( $CR_{total}$ ) under 0.5 or over 2.0, which was outside the scope of the present invention, thereby obtaining  $\alpha+\beta$  type titanium alloy plates having a thickness of 4 mm. Then, the resultant titanium alloy plates were cooled, and then annealed at a temperature of 720° C. for a period of time of an hour, thereby preparing  $\alpha+\beta$  type titanium alloy plates having a thickness of 4 mm outside the scope of the present invention (hereinafter referred to as the "samples for comparison") Nos. 7, 8 and 13.

TABLE 2

| No.                                                                     | Pass schedule                                                                                                                                                                                                                                                                                                                                                                                                                                                                                                                                                                                        | Remark                  |
|-------------------------------------------------------------------------|------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-------------------------|
| 1 (Thickness)<br>Rough-<br>rolling<br>(Thickness)<br>Finish-<br>rolling | $200 \rightarrow 170 \rightarrow 144 \rightarrow 122 \rightarrow 103 \rightarrow 87 \rightarrow 73 \rightarrow 62 \rightarrow 52 \rightarrow 44 \rightarrow 37 \rightarrow 31 \rightarrow 26 \rightarrow 22 \rightarrow 20$<br>$\uparrow (90^\circ \text{-turning})$ <br>$20 \rightarrow 17 \rightarrow 14 \rightarrow 11 \rightarrow 9 \rightarrow 7 \rightarrow 5.5 \rightarrow 4$<br>$\uparrow (90^\circ \text{C. -turning})$  | Sample of the invention |
| 2 (Thickness)<br>Rough-<br>rolling<br>(Thickness)<br>Finish-<br>rolling | $200 \rightarrow 170 \rightarrow 144 \rightarrow 122 \rightarrow 103 \rightarrow 87 \rightarrow 73 \rightarrow 62 \rightarrow 52 \rightarrow 44 \rightarrow 37 \rightarrow 31 \rightarrow 26 \rightarrow 22 \rightarrow 20$<br>$\uparrow (90^\circ \text{-turning})$ <br>$20 \rightarrow 17 \rightarrow 14 \rightarrow 11 \rightarrow 9 \rightarrow 7 \rightarrow 5.5 \rightarrow 4$<br>$\uparrow (90^\circ \text{C. -turning})$  | Sample of the invention |

TABLE 3

| No.                                                                     | Pass schedule                                                                                                                                                                                                                                                                                                                                                                                                                                                                                                                                                                                            | Remark                  |
|-------------------------------------------------------------------------|----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-------------------------|
| 3 (Thickness)<br>Rough-<br>rolling<br>(Thickness)<br>Finish-<br>rolling | $200 \rightarrow 170 \rightarrow 144 \rightarrow 122 \rightarrow 103 \rightarrow 87 \rightarrow 73 \rightarrow 62 \rightarrow 52 \rightarrow 44 \rightarrow 37 \rightarrow 31 \rightarrow 26 \rightarrow 22 \rightarrow 20$<br>$\uparrow (90^\circ \text{-turning})$ <br>$20 \rightarrow 17 \rightarrow 14 \rightarrow 11 \rightarrow 9 \rightarrow 7 \rightarrow 5.5 \rightarrow 4$<br>$\uparrow (90^\circ \text{C. -turning})$  | Sample of the invention |
| 4 (Thickness)<br>Rough-<br>rolling<br>(Thickness)<br>Finish-<br>rolling | $200 \rightarrow 170 \rightarrow 144 \rightarrow 122 \rightarrow 103 \rightarrow 87 \rightarrow 73 \rightarrow 62 \rightarrow 52 \rightarrow 44 \rightarrow 37 \rightarrow 31 \rightarrow 26 \rightarrow 22 \rightarrow 20$ <br>$20 \rightarrow 17 \rightarrow 14 \rightarrow 11 \rightarrow 9 \rightarrow 7 \rightarrow 5.5 \rightarrow 4$                                                                                       | Sample of the invention |

TABLE 4

| No.                       | Pass schedule                                                                                     | Remark                  |
|---------------------------|---------------------------------------------------------------------------------------------------|-------------------------|
| 5 (Thickness)             | 200 → 170 → 144 → 122 → 103 → 87 → 73 → 62 → 52 → 44 → 37 → 31 → 26 → 22 → 20<br>↑ (90° -turning) | Sample of the invention |
| Rough-rolling (Thickness) | under 900 to 850° C. ← → under 850 to 750° C. ← → under 750° C. ← →                               |                         |
| Finish-rolling            | 20 → 17 → 14 → 11 → 9 → 7 → 5.5 → 4<br>↑ (90° C. -turning)                                        |                         |
|                           | under 900 to 850° C. ← → under 850 to 750° C. ← → under 750° C. ← →                               |                         |
| 6 (Thickness)             | 200 → 170 → 144 → 122 → 103 → 87 → 73 → 62 → 52 → 44 → 37 → 31 → 26 → 22 → 20<br>↑ (90° -turning) | Sample of the invention |
| Rough-rolling (Thickness) | under 900 to 850° C. ← → under 850 to 750° C. ← → under 750° C. ← →                               |                         |
| Finish-rolling            | 20 → 17 → 14 → 11 → 9 → 7 → 5.5 → 4<br>↑ (90° C. -turning)                                        |                         |
|                           | under 900 to 850° C. ← → under 850 to 750° C. ← → under 750° C. ← →                               |                         |

TABLE 5

| No.                       | Pass schedule                                                                                                                     | Remark                |
|---------------------------|-----------------------------------------------------------------------------------------------------------------------------------|-----------------------|
| 7 (Thickness)             | 200 → 170 → 144 → 122 → 103 → 87 → 73 → 62 → 52 → 44 → 37 → 31 → 26 → 22 → 20                                                     | Sample for comparison |
| Rough-rolling (Thickness) | under 900 to 850° C. ← → under 850 to 750° C. ← → under 750° C. ← →                                                               |                       |
| Finish-rolling            | 20 → 17 → 14 → 11 → 9 → 7 → 5.5 → 4<br>under 900 to 850° C. ← → under 850 to 750° C. ← → under 750° C. ← →                        |                       |
| 8 (Thickness)             | 200 → 170 → 144 → 122 → 103 → 87 → 73 → 62 → 52 → 44 → 37 → 31 → 26 → 22 → 20<br>↑ (90° -turning)                                 | Sample for comparison |
| Rough-rolling (Thickness) | under 900 to 850° C. ← → under 850 to 750° C. ← → under 750° C. ← →                                                               |                       |
| Finish-rolling            | 20 → 17 → 14 → 11 → 9 → 7 → 5.5 → 4<br>↑ (90° C. -turning)<br>under 900 to 850° C. ← → under 850 to 750° C. ← → under 750° C. ← → |                       |

TABLE 6

| No.                                                              | Pass schedule                                                                                                                                                                           | Remark                  |
|------------------------------------------------------------------|-----------------------------------------------------------------------------------------------------------------------------------------------------------------------------------------|-------------------------|
| 9 (Thickness)<br>Rough-rolling<br>(Thickness)<br>Finish-rolling  | 200 → 170 → 144 → 122 → 103 → 87 → 73 → 62 → 52 → 44 → 37 → 31 → 26 → 22 → 20<br>↑ (90° -turning)<br> | Sample of the invention |
| 10 (Thickness)<br>Rough-rolling<br>(Thickness)<br>Finish-rolling | 200 → 170 → 144 → 122 → 103 → 87 → 73 → 62 → 52 → 44 → 37 → 31 → 26 → 22 → 20<br>↑ (90° -turning)<br>  | Sample of the invention |

TABLE 7

| No.                                                              | Pass schedule                                                                                                                                                                                               | Remark                  |
|------------------------------------------------------------------|-------------------------------------------------------------------------------------------------------------------------------------------------------------------------------------------------------------|-------------------------|
| 11 (Thickness)<br>Finish-rolling                                 | 200 → 170 → 144 → 122 → 103 → 87 → 73 → 62 → 52 → 44 → 37 → 31 → 26 → 22 → 20<br>↑ (90° -turning)<br>                   | Sample of the invention |
| 12 (Thickness)<br>Finish-rolling                                 | 200 → 170 → 144 → 122 → 103 → 87 → 73 → 62 → 52 → 44 → 37 → 31 → 26 → 22 → 20<br>↑ (90° -turning)<br>                   | Sample of the invention |
| 13 (Thickness)<br>Rough-rolling<br>(Thickness)<br>Finish-rolling | 200 → 170 → 144 → 122 → 103 → 87 → 73 → 62 → 52 → 44 → 37 → 31 → 26 → 22 → 20<br>20 → 17 → 14 → 11 → 9 → 7 → 5.5 → 4<br> | Sample for comparison   |

In the samples of the invention Nos. 1 to 3, 5, 6, 9 and 10, and the samples for comparison Nos. 8 and 13, the final rolling direction in the rough-rolling was the same as the first rolling direction in the finish-rolling.

In the sample of the invention No. 4, the turning by right angles of the rolling direction was not effected during the rough-rolling and during the finish-rolling, and the rolling direction in the finish-rolling was at right angles to the rolling direction in the rough-rolling.

In the sample for comparison No. 7, the turning by right angles of the rolling direction was not effected during the rough-rolling and during the finish-rolling, and the rolling direction in the finish-rolling was the same as the rolling direction in the rough-rolling.

In the samples of the invention Nos. 11 and 12, the single-heat rolling was carried out, and the turning by right

angles of the rolling direction was effected once in the middle of the rolling.

A value of the overall cross ratio of rolling ( $CR_{total}$ ) as expressed by the formula (3) described above was determined for each of the samples of the invention and the samples for comparison. A 0.2% proof stress in the L-direction [ $PS(L)$ ] and a 0.2% proof stress in the C-direction [ $PS(C)$ ] were measured by means of a tensile test for each of the samples of the invention and the samples for comparison to determine a value of the ratio [ $PS(L)/PS(C)$ ] of  $PS(L)$  to  $PS(C)$ . The values thus determined are shown in Table 8.

TABLE 8

| No. | CR <sub>total</sub><br>according to<br>formula(3) | 0.2% proof<br>stress in<br>L-direction<br>[PS(L)] | 0.2% proof<br>stress in<br>C-direction<br>[PS(C)] | PS(L)<br>PS(C) | Remark                     |
|-----|---------------------------------------------------|---------------------------------------------------|---------------------------------------------------|----------------|----------------------------|
| 1   | 0.932                                             | 899 MPa                                           | 870 MPa                                           | 1.022          | Sample of<br>the invention |
| 2   | 1.614                                             | 881 MPa                                           | 1032 MPa                                          | 0.854          |                            |
| 3   | 0.625                                             | 897 MPa                                           | 879 MPa                                           | 1.020          |                            |
| 4   | 0.564                                             | 907 MPa                                           | 880 MPa                                           | 1.031          |                            |
| 5   | 0.587                                             | 907 MPa                                           | 884 MPa                                           | 1.026          |                            |
| 6   | 1.099                                             | 859 MPa                                           | 903 MPa                                           | 0.951          |                            |
| 7   | 26.234                                            | 674 MPa                                           | 1028 MPa                                          | 0.656          | Sample for<br>comparison   |
| 8   | 3.090                                             | 786 MPa                                           | 981 MPa                                           | 0.801          |                            |
| 9   | 0.571                                             | 1007 MPa                                          | 881 MPa                                           | 1.143          | Sample of<br>the invention |
| 10  | 1.080                                             | 887 MPa                                           | 916 MPa                                           | 0.957          |                            |
| 11  | 1.204                                             | 880 MPa                                           | 965 MPa                                           | 0.911          |                            |
| 12  | 0.909                                             | 910 MPa                                           | 881 MPa                                           | 1.033          |                            |
| 13  | 0.284                                             | 1044 MPa                                          | 822 MPa                                           | 1.270          | Sample for<br>comparison   |

As is clear from Table 8, in any of the samples of the invention Nos. 1 to 6 and 9 to 12, in which the value of the overall cross ratio of rolling (CR<sub>total</sub>) determined by means of the formula (3) was within a range of from 0.5 to 2.0, which was within the scope of the present invention, the value of the ratio [PS(L)/PS(C)] of the 0.2% proof stress in the L-direction [PS(L)] to the 0.2% proof stress in the C-direction [PS(C)], was within a range of from 0.80 to 1.20. Therefore, any of the  $\alpha+\beta$  type titanium alloy plates manufactured according to the method of the present invention was excellent in isotropy with a small anisotropy in strength.

In contrast, in any of the samples for comparison Nos. 7, 8 and 13, in which the value of the overall cross ratio of rolling (CR<sub>total</sub>) determined by means of the formula (3) was under 0.5 or over 2.0, which was outside the scope of the present invention, the value of the ratio [PS(L)/PS(C)] of the 0.2% proof stress in the L-direction [PS(L)] to the 0.2% proof stress in the C-direction [PS(C)], was under 0.80 or over 1.20. Therefore, any of the  $\alpha+\beta$  type titanium alloy

An alloy comprising a Ti-6Al-4V alloy was employed as an  $\alpha+\beta$  type titanium alloy. Since this titanium alloy has a  $\beta$ -transformation temperature ( $T\beta$  °C.) of 1,000° C., the temperature region of the hot-rolling of the titanium alloy slab was divided, in Example 2, into three rolling temperature regions of (1) from under 1,000° C. to 950° C., (2) from under 950° C. to 850° C., and (3) under 850° C.

- 10 While keeping a value of the overall cross ratio of rolling (CR<sub>total</sub>) within a range of from 0.5 to 2.0, an  $\alpha+\beta$  type titanium alloy slab having a thickness of 200 mm and the above-mentioned chemical composition, was rough-rolled and then finish-rolled in accordance with a pass schedule shown in Table 9 in the same manner as in the sample of the invention No. 1, thereby obtaining an  $\alpha+\beta$  type titanium alloy plate having a thickness of 4 mm. Then, the resultant titanium alloy plate was cooled, and then annealed at a temperature of 720° C. for a period of time of an hour.
- 15 thereby preparing an  $\alpha+\beta$  type titanium alloy plate having a thickness of 4 mm within the scope of the present invention (hereinafter referred to as the "sample of the invention") No. 14.

Then, for comparison purposes, an  $\alpha+\beta$  type titanium alloy slab having the same chemical composition and the same thickness as those in the sample of the invention No. 14, was rough-rolled and then finish-rolled in accordance with a pass schedule shown in Table 9 in the same manner as described above, while keeping a value of the overall cross ratio of rolling (CR<sub>total</sub>) under 0.5 or over 2.0, which was outside the scope of the present invention, thereby obtaining an  $\alpha+\beta$  type titanium alloy plate having a thickness of 4 mm. Then the resultant titanium alloy plate was cooled, and then annealed at a temperature of 720° C. for a period of time of an hour, thereby preparing an  $\alpha+\beta$  type titanium alloy plate having a thickness of 4 mm outside the scope of the present invention (hereinafter referred to as the "sample for comparison") No. 15.

TABLE 9

| No.                                                                      |                                                                                                      | Pass schedule | Remark                     |
|--------------------------------------------------------------------------|------------------------------------------------------------------------------------------------------|---------------|----------------------------|
| 14 (Thickness)<br>Rough-<br>rolling<br>(Thickness)<br>Finish-<br>rolling | 200 → 170 → 144 → 122 → 103 → 87 → 73 → 62 → 52 → 44 → 37 → 31 → 26 → 22 → 20<br>↑ (90° -turning)    |               | Sample of the<br>invention |
|                                                                          |                  |               |                            |
| 15 (Thickness)<br>Rough-<br>rolling<br>(Thickness)<br>Finish-<br>rolling | 200 → 170 → 144 → 122 → 103 → 87 → 73 → 62 → 52 → 44 → 37 → 31 → 26 → 22 → 20<br>↑ (90° C. -turning) |               | Sample for<br>comparison   |
|                                                                          |                  |               |                            |

plates manufactured according to the method outside the scope of the present invention had a large anisotropy in strength.

65 In the sample of the invention No. 14, the final rolling direction in the rough-rolling was the same as the first rolling direction in the finish-rolling.

In the sample for comparison No. 15, the turning by right angles of the rolling direction was not effected during the rough-rolling and during the finish-rolling, and the rolling direction in the finish-rolling was the same as the rolling direction in the rough-rolling.

A value of the overall cross ratio of rolling ( $CR_{total}$ ) as expressed by the formula (3) described above was determined for each of the samples of the invention and the samples for comparison. A 0.2% proof stress in the L-direction [PS(L)] and a 0.2% proof stress in the C-direction [PS(C)] were measured by means of a tensile test for each of the samples of the invention and the samples for comparison to determine a value of the ratio [PS(L)/PS(C)] of PS(L) to PS(C). The values thus determined are shown in Table 10.

TABLE 10

| No. | $CR_{total}$<br>according to<br>formula(3) | 0.2% proof<br>stress in | 0.2% proof<br>stress in | PS(L)<br>PS(C) | Remark                     |
|-----|--------------------------------------------|-------------------------|-------------------------|----------------|----------------------------|
|     |                                            | L-direction<br>[PS(L)]  | C-direction<br>[PS(C)]  |                |                            |
| 14  | 0.932                                      | 1004 MPa                | 981 MPa                 | 1.023          | Sample of<br>the invention |
| 15  | 26.234                                     | 743 MPa                 | 1133 MPa                | 0.656          | Sample for<br>comparison   |

As is clear from Table 10, in the sample of the invention No. 14, in which the value of the overall cross ratio of rolling ( $CR_{total}$ ) determined by means of the formula (3) was within a range of from 0.5 to 2.0, which was within the scope of the present invention, the value of the ratio [PS(L)/PS(C)] of the 0.2% proof stress in the L-direction [PS(L)] to the 0.2% proof stress in the C-direction [PS(C)], was within a range of from 0.80 to 1.20. Therefore, the  $\alpha+\beta$  type titanium alloy plate manufactured according to the method of the present invention, was excellent in isotropy with a small anisotropy in strength.

In contrast, in the sample for comparison No. 15, in which the value of the overall cross ratio of rolling ( $CR_{total}$ ) determined by means of the formula (3) was over 2.0, which was outside the scope of the present invention, the value of the ratio [PS(L)/PS(C)] of the 0.2% proof stress in the L-direction [PS(L)] to the 0.2% proof stress in the C-direction [PS(C)], was under 0.80. Therefore, the  $\alpha+\beta$  type titanium alloy plate manufactured according to the method outside the scope of the present invention had a large anisotropy in strength.

According to the method of the present invention, as described above in detail, it is possible to efficiently manufacture an  $\alpha+\beta$  type titanium alloy plate excellent in isotropy with a small anisotropy in strength, thus providing many industrially useful effects.

What is claimed is:

1. A method for manufacturing an  $\alpha+\beta$  titanium alloy plate having a small anisotropy in strength by subjecting an  $\alpha+\beta$  titanium alloy slab to a hot-rolling, which comprises: said hot-rolling comprising a cross-rolling which comprises a hot-rolling in an L-direction and a hot-rolling

in a C-direction, said L-direction being a final rolling direction in said hot-rolling and said C-direction being a direction at right angles to said L-direction; and

controlling said cross-rolling so that a value of an overall cross ratio of rolling ( $CR_{total}$ ) determined by means of the following formula is kept within a range of from 0.5 to 2.0:

$$CR_{total} = (CR_1)^{0.6} \times (CR_2)^{0.8} \times (CR_3)^{1.0}$$

where,

$CR_{total}$ : overall cross ratio of rolling,

$CR_1$ : cross ratio of rolling within a rolling temperature region of from under  $T\beta$  °C. to  $T\beta$  °C.-50° C.,

$CR_2$ : cross ratio of rolling within a rolling temperature region of from under  $T\beta$  °C.-50° C. to  $T\beta$  °C.-150° C.,

$CR_3$ : cross ratio of rolling within a rolling temperature region of under  $T\beta$  °C.-150° C., and

$T\beta$  °C.:  $\beta$ -transformation temperature of an  $\alpha+\beta$  titanium alloy.

2. A method as claimed in claim 1, wherein:

said cross-rolling comprises a cross-rolling in a rough-rolling and a cross-rolling in a finish-rolling; and

controlling said cross-rolling so that a value of an overall cross ratio of rolling ( $CR_{total}$ ) determined by means of the following formula is kept within a range of from 0.5 to 2.0:

$$CR_{total} = [(CR_1)^{0.6} \times (CR_2)^{0.8} \times (CR_3)^{1.0} \text{ in rough-rolling}] \times [(CR_1)^{0.6} \times (CR_2)^{0.8} \times (CR_3)^{1.0} \text{ in finish-rolling}].$$

3. A method as claimed in claim 1 or 2, wherein:

a value of a ratio [PS(L)/PS(C)] of a 0.2% proof stress in said L-direction [PS(L)] to a 0.2% proof stress in said C-direction [PS(C)] is within a range of from 0.80 to 1.20.

4. A method as claimed in claim 1 or 2, wherein:

said  $\alpha+\beta$  titanium alloy slab comprises a Ti-4.5Al-3V-2Mo-2Fe alloy.

5. A method as claimed in claim 1 or 2, wherein:

said  $\alpha+\beta$  titanium alloy slab comprises a Ti-6Al-4V alloy.

6. A method as claimed in claim 3, wherein:

said  $\alpha+\beta$  titanium alloy slab comprises a Ti-4.5Al-3V-2Mo-2Fe alloy.

7. A method as claimed in claim 3, wherein:

said  $\alpha+\beta$  titanium alloy slab comprises a Ti-6Al-4V alloy.

\* \* \* \* \*